

1

2,984,624

## LUBRICATING OIL THICKENED TO A GREASE WITH A MIXTURE OF A 1,3,5-TRIAZINE COMPOUND AND AN ORGANOPHILIC SILICEOUS COMPOUND

Robert E. Halter, Verona, and Joseph J. McGrath, Monroeville, Pa., assignors to Gulf Research & Development Company, Pittsburgh, Pa., a corporation of Delaware

No Drawing. Filed July 31, 1959, Ser. No. 830,718

15 Claims. (Cl. 252—28)

This invention relates to improved lubricating compositions and more particularly to lubricants suitable for high temperature lubrication comprising a lubricating oil thickened primarily with certain high melting symmetrical (s) triazines, specifically those melting above about 400° F. (205° C.).

The trend in design of modern aircraft has accentuated the need for greases which will lubricate anti-friction bearings operating at high rotational speeds and high temperatures. While considerable progress has been made in recent years in producing improved aircraft greases some difficulty has been encountered in producing a grease which will effectively lubricate bearings operating at high rotational speeds and high temperatures for prolonged periods of time. Conventional aircraft greases currently available have failed to meet the stringent requirements on such a lubricant.

We have discovered that a lubricating composition having improved lubricating characteristics for an extended period of time when used to lubricate bearings operating at an elevated temperature under high rotational speeds can be obtained by incorporating into a lubricating oil in oil thickening proportions a mixture of a symmetrical triazine, i.e., 1,3,5-triazine, compound melting above about 205° C. having the following formula:



wherein R and R<sub>1</sub> are selected from the group consisting of hydrogen, alkyl, aryl, alkaryl, aralkyl, cyanoalkyl, pyridyl, amino, hydroxy and mercapto radicals, R and R<sub>1</sub> being unlike radicals when selected from the group consisting of amino, hydroxy and mercapto radicals and a secondary organophilic siliceous oil thickening agent. Thus, the improved lubricating composition of our invention comprises a dispersion in a lubricating oil of a sufficient amount to thicken the lubricating oil to a grease consistency of a mixture of a 1,3,5-triazine melting above about 205° C. of the type designated by the above structural formula and an organophilic siliceous oil thickening agent.

2

It will be noted that R and R<sub>1</sub> can be the same or different radicals when selected from the group consisting of hydrogen, alkyl, aryl, alkaryl, aralkyl, cyanoalkyl and pyridyl radicals provided, of course, that the melting point of the compound is at least 205° C. When R and R<sub>1</sub> are selected from the group consisting of amino, hydroxy and mercapto radicals, the radicals should not all be the same. For example, we do not intend to include compounds such as cyanuric acid (s-triazinetriol) or melamine (2,4,6-triamino-s-triazine).

An especially preferred group of triazine compounds for the purpose of our invention includes those compounds wherein each of the R radicals is an amino radical, that is, a guanamine derivative. Preferred guanamine derivatives are those wherein R<sub>1</sub> is selected from the group consisting of hydrogen, alkyl (e.g., methyl, ethyl, propyl and n-butyl), aryl (e.g., phenyl and naphthyl), alkaryl (e.g., tolyl), aralkyl (e.g., benzyl), cyanoalkyl (e.g., cyanoethyl, cyanobutyl and cyanoctyl), pyridyl, hydroxy and mercapto radicals. When R<sub>1</sub> in the guanamine derivatives is an alkyl radical, it preferably is selected from the group consisting of methyl, ethyl, propyl and n-butyl radicals in order to give a compound having a melting point above about 205° C. When R<sub>1</sub> is isobutyl or a higher alkyl radical the melting point of the resulting substituted guanamine is below 205° C. While compounds melting below 205° C. can be used to produce grease compositions for use at temperatures below 400° F., such compounds are not satisfactory thickening agents for grease compositions used to lubricate bearings operating at high rotational speeds at temperatures of 400° F. and higher for prolonged periods of time. When R<sub>1</sub> in the guanamine derivatives is an alkaryl or an aralkyl radical, the alkyl portion of the alkaryl and aralkyl radicals preferably contains not more than 2 carbon atoms. When R<sub>1</sub> in the preferred guanamine derivatives is a cyanoalkyl radical, the alkyl portion of the cyanoalkyl radical can contain as many as 8 carbon atoms and still give a compound melting above 205° C.

Illustrative of the preferred guanamine derivatives which can be used in the present invention are the following:

- 2,4-diamino-1,3,5-triazine
- 2,4-diamino-6-methyl-1,3,5-triazine
- 50 2,4-diamino-6-ethyl-1,3,5-triazine
- 2,4-diamino-6-propyl-1,3,5-triazine
- 2,4-diamino-6-n-butyl-1,3,5-triazine
- 2,4-diamino-6-phenyl-1,3,5-triazine
- 55 2,4-diamino-6- $\alpha$ -naphthyl-1,3,5-triazine
- 2,4-diamino-6- $\beta$ -naphthyl-1,3,5-triazine
- 2,4-diamino-6-m-tolyl-1,3,5-triazine
- 2,4-diamino-6-p-tolyl-1,3,5-triazine
- 2,4-diamino-6-benzyl-1,3,5-triazine
- 60 2,4-diamino-6-cyanoethyl-1,3,5-triazine
- 2,4-diamino-6-cyanobutyl-1,3,5-triazine
- 2,4-diamino-6-cyanoctyl-1,3,5-triazine
- 2,4-diamino-6-pyridyl-1,3,5-triazine

2,4-diamino-6-hydroxy-1,3,5-triazine  
2,4-diamino-6-mercaptop-1,3,5-triazine

While the guanamine derivatives of the above type are all effective thickeners for the preparation of high temperature greases, it is not to be implied that all serve with equal efficiency, since the various compounds may vary to some extent depending upon the nature and severity of the service to which they are subjected. Those guanamine derivatives which contain an aryl radical, such as a phenyl radical, because of the increased thermal stability contributed to the compounds by such a radical are especially preferred. Thus, benzoguanamine is an especially preferred primary thickening agent in the grease compositions of the present invention.

The amount of the combined 1,3,5-triazine and the organophilic siliceous material which we use is an amount sufficient to thicken the lubricating oil to a grease consistency. In general, this amount comprises about 10 to about 60 percent by weight of the total composition. The weight ratio of the 1,3,5-triazine compound to the organophilic siliceous material will vary depending upon the characteristics desired in the ultimate composition. In general, however, the ratio of the 1,3,5-triazine compound to the organophilic siliceous material is between about 1:1 and about 20:1.

The amount of the 1,3,5-triazine compound used may vary over wide limits depending upon the particular oil with which the triazine compound is to be blended and upon the properties desired in the final lubricating composition. While as much as 50 percent by weight of the total composition may comprise the triazine compound, we prefer to use smaller amounts, that is, in the order of about 10 to 40 percent by weight. It should be understood, however, that, depending upon the consistency of the composition desired and upon the organophilic siliceous material used in combination therewith, less than 10 percent or more than 50 percent of the triazine compound may be employed.

The 1,3,5-triazine compounds can be prepared according to known chemical procedures. Neither the compounds per se nor their preparation constitutes any portion of the invention. For example, a 2-amino-4,6-dialkyl-1,3,5-triazine can be prepared by reacting a nitrile with guanidine. A 2,6-diamino-4-alkyl-1,3,5-triazine can be prepared by reacting alkyl biguanides with acylating agents in the presence of alkali. Acetoguanamine (2,4-diamino-6-methyl-1,3,5-triazine) having a melting point of 271° to 273° C. can be prepared by reacting dicyandiamide and acetonitrile in the presence of piperidine. Benzoguanamine (2,4-diamino-6-phenyl-1,3,5-triazine) having a melting point of 222° C. can be prepared by reacting dicyandiamide and benzonitrile in the presence of piperidine. 2,4-diamino-6-(2'-naphthyl)-1,3,5-triazine having a melting point of 240° C. can be prepared by reacting beta-naphthonitrile and dicyandiamide in the presence of piperidine. 2,4-diamino-6-benzyl-1,3,5-triazine having a melting point of 232° C. can be prepared by reacting dicyandiamide and benzylcyanide in the presence of piperidine. The preparation of some of the 1,3,5-triazines is more fully described in U.S. Patent No. 2,527,314, issued October 24, 1950, to Johnstone S. Mackay; U.S. Patent No. 2,302,162, issued November 17, 1942, to Werner Zerweck et al.; and U.S. Patent No. 2,408,694, issued October 1, 1946, to John Kenson et al.

The following illustrative example will serve to demonstrate the preparation of a pyridyl 1,3,5-triazine which can be used in preparing a grease composition of the present invention.

## EXAMPLE I

## 2,4-dihydroxy-6-pyridyl-1,3,5-triazine

Cyanuric chloride (18.5 gm., 0.1 mole), pyridine (100 ml.) and water (500 ml.) were stirred at room temperature for thirty minutes and then filtered. The filtrate was concentrated on a water bath to give a product comprising 2,4-dihydroxy-6-pyridyl-1,3,5-triazine having a melting point above 400° C. (752° F.).

It should be understood that the symmetrical (s) triazine compounds can contain other substituents provided, of course, that said other substituents do not adversely affect the beneficial oil thickening properties of the s-triazine compounds.

The organophilic siliceous materials which we employ in the lubricating composition of this invention are exemplified by bentonite-organic base compounds known commercially as "Bentones" and finely divided organophilic siliceous solids such as the esterified siliceous solids known commercially as "Estersils." The amount of the organophilic siliceous material employed may vary over wide limits depending upon the particular compound employed, the particular oil with which the siliceous compound is blended and the properties desired in the ultimate composition. While the organophilic siliceous material may comprise as much as 20 percent by weight of the total composition, we prefer to use smaller amounts, that is, in the order of about 1 to about 10 percent by weight. It should be understood, however, that depending upon the consistency of the composition desired and upon the triazine content of the composition less than 1 percent or more than 10 percent of the organophilic siliceous material can be employed.

Typical bentonite-organic base compounds employed in accordance with the invention are compounds composed of a montmorillonite mineral in which at least a part of the cation content of the mineral has been replaced by an organic base. Clays that swell at least to some extent on being contacted with water and contain as a primary constituent a mineral of the group known as montmorillonites are generally referred to as bentonites. Such clays, which contain exchangeable alkali metal atoms either naturally or after treatment, constitute the raw materials employed in making the bentonite-organic base compounds used in the compositions of this invention. So far as known, all naturally occurring montmorillonites contain some magnesium and certain of them, as exemplified by Hector clay, contain such a high percentage of magnesium that they largely have magnesium in place of the aluminum content characteristic of the more typical montmorillonites.

The bentonite-organic base compounds are preferably prepared as described in U.S. Patent No. 2,033,856, issued March 10, 1936, by bringing together the bentonite and the organic base in the presence of aqueous mineral acid to effect base exchange. The organic bases should preferably be titratable with mineral acids. Among these reactive bases are many alkaloids, and cyclic, aliphatic, and heterocyclic amines. The bentonite-organic base compounds used in preparing the lubricating compositions of this invention are preferably those prepared by bringing together a bentonite clay and such organic bases as aliphatic amines, their salts, and quaternary ammonium salts. Examples of such amines and salts are: decylamine, dodecylamine, tetradecylamine, hexadecylamine, octadecylamine, hexadecyl ammonium acetate, octadecyl ammonium acetate, dimethyldioctyl ammonium acetate, dimethyldidodecyl ammonium acetate, dimethyldodecylhexadecyl ammonium acetate, dimethyl-

dicetyl ammonium acetate, dimethylhexadecyloctadecyl ammonium acetate, dimethyldioctadecyl ammonium acetate, and the corresponding chlorides and quaternary ammonium chlorides. The organic bases employed should be such as to impart substantial organophilic properties to the resulting compounds. The preferred bentonite compounds are prepared from quaternary ammonium compounds in which the N-substituents are aliphatic groups containing at least one alkyl group with a total of at least 10 to 12 carbon atoms. When aliphatic amines are used they preferably contain at least one alkyl group containing at least 10 to 12 carbon atoms.

While the long chain aliphatic amine bentonite compounds are readily dispersible in practically all oil bases, dispersion of the short or single chain aliphatic amine bentonite compounds, in the oil, particularly mineral oils and synthetic oils other than ester lubricants, can be facilitated by the use of one or more solvating agents. Suitable solvating agents are polar organic compounds such as organic acids, esters, alcohols, ethers, ketones, and aldehydes, especially low molecular weight compounds of these classes. Examples of suitable solvating agents are: ethyl acetate, acetic acid, acetone, methyl alcohol, ethyl alcohol, benzoyl chloride, butyl stearate, cocoanut oil, cyclohexanone, ethylene dichloride, ethyl ether, furfural, isoamyl acetate, methyl ethyl ketone, and nitrobenzene. In cases where the use of a solvating agent is desirable for effecting more rapid and more complete dispersion of the organic bentonite compound in the oil, ordinarily only a relatively small amount of such agent may be necessary. However, as much as about 50 percent by weight based on the amount of the bentonite compound can be used.

Typical estersils employed in accordance with the invention are described in U.S. Patent No. 2,657,149, issued October 27, 1953, to R. K. Iler. The estersils are organophilic solids made by chemically reacting primary or secondary alcohols with certain siliceous solids. In brief, the estersils are powders or pulverulent materials the internal structure or "substrate" of which have an average specific surface area of from 1 to 900 square meters per gram. The substrate has a surface of silica which is coated with —OR' groups, the coating of —OR' groups being chemically bound to the silica. R' is a hydrocarbon radical of a primary or secondary alcohol containing from 2 to 18 carbon atoms. The carbon atom attached to the oxygen is also attached to hydrogen.

The estersil substrates are solid inorganic siliceous materials which contain substantially no chemically bound organic groups prior to esterification. The substrates are in a supercolloidal state of subdivision, indicating that whatever discrete particles are present are larger than colloidal size. In general, the supercolloidal substrates have at least one dimension of at least 150 millimicrons. The supercolloidal particles may be aggregates of ultimate units which are colloidal in size.

The estersils which we employ are advantageously those in which the ultimate units have an average diameter of 8 to 10 millimicrons. The substrates advantageously have specific surface areas of at least 25 square meters per gram and preferably at least 200 square meters per gram.

The estersils made from most alcohols become organophilic when they contain more than about 80 ester groups per 100 square millimicrons of surface of internal structure. They become more organophilic as the ester groups increase. Thus, the products which contain 100 ester groups per 100 square millimicrons of substrate surface are more organophilic than those that contain only 80 ester groups. When the estersils contain at least

200 ester groups per 100 square millimicrons of substrate surface, the estersils not only are organophilic but also are hydrophobic. Thus, the more highly esterified products are particularly desirable where the lubricant made therefrom comes in contact with water. When C<sub>3</sub> to C<sub>6</sub> alcohols are used in preparing the estersils, the estersils may contain from 300 to 400 ester groups per 100 square millimicrons of substrate surface. Thus, a preferred group of estersils are those prepared from the C<sub>3</sub> to C<sub>6</sub> alcohols. The estersils, as noted above, are powders or pulverulent materials. The estersil powders are exceedingly fine, light and fluffy. The bulk density of preferred estersils is in the order of 0.15 to 0.20 gram per cubic centimeter at 3 pounds per square inch and in the order of about 0.30 gram per cubic centimeter at 78 pounds per square inch. The estersils are available commercially and thus the estersils per se and their preparation constitute no part of this invention.

20 The lubricating oil in which the triazine compound and the secondary thickening agent are incorporated is preferably a lubricant of the type best suited for the particular use for which the ultimate composition is designed. Since many of the properties possessed by the lubricating oil are imparted to the ultimate lubricating composition, we advantageously employ an oil which is thermally stable at the contemplated lubricating temperature. Some mineral oils, especially hydrotreated mineral oils, are sufficiently stable to provide a lubricating base for preparing lubricants to be used under moderately elevated temperatures. Where temperatures in the order of 400° F. and above are to be encountered, synthetic oils form a preferred class of lubricating bases 30 because of their high thermal stability. By the term "synthetic oil" we mean an oil of non-mineral origin. The synthetic oil can be an organic ester which has a majority of the properties of a hydrocarbon oil of lubricating grade such as di-2-ethylhexyl sebacate, dioctyl phthalate and dioctyl azelate. Instead of an organic ester, we can use polymerized olefins, copolymers of alkylene glycols and alkylene oxides, polyorgano siloxanes and the like.

35 40 45 The liquid polyorgano siloxanes because of their exceedingly high thermal stability form a preferred group of synthetic oils to which the triazine compound and organophilic siliceous materials are added. These polyorgano siloxanes are known commercially as silicones and are made up of silicon and oxygen atoms wherein the silicon atoms may be substituted with alkyl, aryl, alkaryl, aralkyl and cycloalkyl radicals. Exemplary of such compounds are the dimethyl silicone polymers, diethyl silicone polymers, ethyl-phenyl silicone polymers and methyl-phenyl silicone polymers.

If desired, a blend of oils of suitable viscosity may be employed as the lubricating oil base instead of a single oil by means of which any desired viscosity may be secured. Therefore, depending upon the particular use for which the ultimate composition is designed, the lubricating oil base may be a mineral oil, a synthetic oil, or a mixture of mineral and/or synthetic oils. The lubricating oil content of the compositions prepared according to this invention comprises about 40 to about 90 percent by weight of the total composition.

In compounding the compositions of the present invention, various mixing and blending procedures may be used. In a preferred embodiment of the invention, the lubricating oil, the triazine compound and the secondary thickener together with a solvating agent and conventional lubricant additives, if desired, are mixed together at room temperature for a period of 10 to 30 minutes to 70 75 form a slurry. During this initial mixing period some

thickening is evidenced. Some lumps may be formed. The slurry thus formed is then subjected to a conventional milling operation in a ball mill, a colloid mill, homogenizer or similar device used in compounding greases to give the desired degree of dispersion. In the illustrative compositions of this invention, the slurry was passed twice, by means of a pump, through a Premier Colloid Mill set at a stator-rotor clearance of 0.002 inch. Maximum thickening occurred on the second pass through the mill.

The lubricating composition of this invention can contain conventional lubricant additives, if desired, to improve other specific properties of the lubricant without departing from the scope of the invention. Thus, the lubricating composition can contain a filler, a corrosion and rust inhibitor, an extreme pressure agent, an antioxidant, a metal deactivator, a dye, and the like. Whether or not such additives are employed and the amounts thereof depend to a large extent upon the severity of the conditions to which the composition is subjected and upon the stability of the lubricating oil base in the first instance. Since the polyorgano siloxanes, for example, are in general more stable than mineral oils, they require the addition of very little, if any, oxidation inhibitor. When such conventional additives are used they are generally added in amounts between about 0.01 and 5 percent by weight based on the weight of the total composition.

In order to illustrate the lubricating characteristics at an elevated temperature and high rotational speeds, grease compositions of the invention were subjected to the test procedure outlined by the Coordinating Research Council Tentative Draft (July 1954), "Research Technique for the Determination of Performance Characteristics of Lubricating Grease in Antifriction Bearings at Elevated Temperatures," CRC Designation L-35. According to this procedure, 3 grams of the grease to be tested are placed in a bearing assembly containing an eight-ball SAE No. 204 ball bearing. The bearing assembly which is mounted on a horizontal spindle is subjected to a radial load of 5 pounds. The portion of the spindle upon which the test bearing assembly is located is encased in a thermostatically controlled oven. By this means the temperature of the bearing can be maintained at a desired elevated temperature which in the tests reported hereinafter was 400° F. The spindle is driven by a constant belt-tension motor drive assembly, capable of giving spindle speeds up to 10,000 revolutions per minute. The spindle is operated on a cycling schedule consisting of a series of periods, each period consisting of 20 hours running time and 4 hours shutdown time. The test continues until the lubricant fails. The lubricant is considered to have failed when any one of the following conditions occurs, (1) spindle input power increases to a value approximately 300 percent above the steady state condition at the test temperature; (2) an increase in temperature at the test bearing of 20° F. over the test temperature during any portion of a cycle; or (3) the test bearing locks or the drive belt slips at the start or during the test cycle. The results of a more severe test using Pope spindles and an MRC 204 S-17 bearing at 400° F. and 20,000 revolutions per minute are also reported in Table I.

The oil used in preparing the lubricating compositions summarized in Table I was a synthetic oil known commercially as DC 550 Fluid marketed by Dow-Corning Corporation. This fluid is a methylphenylsiloxane polymer having as typical characteristics a viscosity at 100° F. of 300 to 400 SUS, a viscosity-temperature coefficient

of 0.75, a freezing point of -54° F., a flash point of 600° F. and a specific gravity 25° C./25° C. of 1.08.

In preparing the lubricating compositions, the oil, the triazine and the dimethyldicetyl ammonium bentonite were mixed at room temperature for a period of 10 to 30 minutes. The slurry thus formed was passed twice through a Premier Colloid Mill set at a stator-rotor clearance of 0.002 inch. The thickened lubricating compositions thus prepared had the following approximate make-up and properties.

TABLE I

|    | Composition, Percent By Weight                                                                                          | A    | B    | C    | D    | E    |
|----|-------------------------------------------------------------------------------------------------------------------------|------|------|------|------|------|
| 20 | Lubricating Oil, DC 550 Fluid                                                                                           | 63.0 | 67.4 | 67.4 | 68.9 | 63.0 |
| 25 | Primary Thickener: Benzoguanamine (2,4-diamino-6-phenyl-1,3,5-triazine) Ammelide (2,4-dihydroxy-6-amino-1,3,5-triazine) | 33.0 | 29.1 | 29.1 |      |      |
| 30 | Ammeline (2,4-diamino-6-hydroxy-1,3,5-triazine) 2,4-Dihydroxy-6-pyridyl-1,3,5-triazine                                  |      |      | 27.5 |      | 33.0 |
| 35 | 2,4-Dimercapto-6-amino-1,3,5-triazine                                                                                   |      |      |      |      |      |
| 40 | Secondary Thickener: Dimethyldicetyl ammonium bentonite                                                                 | 4.0  | 3.5  | 3.5  | 3.6  | 4.0  |
| 45 | Inspection: Penetration (ASTM D217-52T) Unworked                                                                        | 275  | 272  | 253  | 242  | 233  |
| 50 | Worked                                                                                                                  | 302  | 287  | 287  | 298  | 251  |
| 55 | Dropping Point, °F. (ASTM D566-42) Performance Life, hrs.: 10,000 r.p.m. at 400° F.                                     | 450+ | 450+ | 450+ | 450+ | 450+ |
| 60 | 20,000 r.p.m. at 400° F.                                                                                                | 734  | 347  | 194  | 285  | 557  |
| 65 |                                                                                                                         | 112  | 323  | 161  | 253  | 94   |

The long performance life of the compositions of the invention at high rotational speeds and a high temperature is self evident from the above data.

Other lubricating compositions within the scope of the invention are illustrated in Table II. G. E. Silicone 81717 is marketed by General Electric Company and is a water-white to amber liquid polymer of the general formula



It has a viscosity at -65° F. of 3487 centistokes, at 0° 210° F. of 22 centistokes and at 700° F. of 1.9 centistokes.

Estersil GT is marketed by E. I. du Pont de Nemours and Company and consists of an amorphous silica coated with approximately 340 butoxy groups per 100 square millimicrons of surface. The product is a white granular solid comprising 88 to 89 percent  $\text{SiO}_2$  having an ultimate particle size of 8 to 10 millimicrons. The surface area comprises about 285 to 335 square meters per gram. The product has a pH in a 50-50 methanol-water mixture of 8.0 to 9.0 and a bulk density of 19 to 20 pounds per cubic foot.

TABLE II

| Composition, Percent By Weight                         | F   | G   | H   | I   | J   | K    | L   | M   | N   | O   | P   | Q   | R   | S   | T   |
|--------------------------------------------------------|-----|-----|-----|-----|-----|------|-----|-----|-----|-----|-----|-----|-----|-----|-----|
| Lubricating Oil:                                       |     |     |     |     |     |      |     |     |     |     |     |     |     |     |     |
| DC 650 Fluid.....                                      | 64  | 70  | 70  | 64  | 64  | 47.5 | 70  | 80  | 70  | 70  | 60  | 60  | 70  | 64  | 60  |
| G.E. Silicone 81717.....                               |     |     |     |     |     |      |     |     |     |     |     |     |     |     |     |
| Di-2-ethylhexyl sebacate.....                          |     |     |     |     |     |      |     |     |     |     |     |     |     |     |     |
| Primary Thickener:                                     |     |     |     |     |     |      |     |     |     |     |     |     |     |     |     |
| 2,4-diamino-1,3,5-triazine.....                        | 32  |     |     |     |     |      |     |     |     |     |     | 35  |     |     |     |
| 2,4-diamino-6-methyl-1,3,5-triazine.....               |     | 24  |     |     |     |      |     |     |     |     |     |     |     |     |     |
| 2,4-diamino-6-ethyl-1,3,5-triazine.....                |     |     | 24  |     |     |      |     |     |     |     |     |     | 30  |     |     |
| 2,4-diamino-6-n-butyl-1,3,5-triazine.....              |     |     |     | 30  |     |      |     |     |     |     |     |     |     | 25  |     |
| 2,4-diamino-6-benzyl-1,3,5-triazine.....               |     |     |     |     | 32  |      |     |     |     |     |     |     |     |     |     |
| 2,4-diamino-6-p-tolyl-1,3,5-triazine.....              |     |     |     |     |     | 50   |     |     |     |     |     |     |     |     |     |
| 2,4-diamino-6-naphthyl-1,3,5-triazine.....             |     |     |     |     |     |      | 20  |     |     |     |     |     |     | 32  |     |
| 2,4-diamino-6-cyanoethyl-1,3,5-triazine.....           |     |     |     |     |     |      |     | 10  |     |     |     |     |     |     |     |
| 2,4-diamino-6-cyanobutyl-1,3,5-triazine.....           |     |     |     |     |     |      |     |     | 20  |     |     |     |     |     | 36  |
| 2,4-diamino-6-cyanoctyl-1,3,5-triazine.....            |     |     |     |     |     |      |     |     |     | 25  |     |     |     |     |     |
| Secondary Thickener:                                   |     |     |     |     |     |      |     |     |     |     |     |     |     |     |     |
| Dimethylidicylammonium bentonite.....                  | 4   |     |     |     |     |      |     | 10  | 10  | 10  | 5   |     |     |     | 4   |
| Dimethylidodecylammonium bentonite.....                |     | 6   |     |     |     |      |     |     |     |     |     |     |     |     |     |
| Dimethylidoclammonium bentonite.....                   |     |     | 6   |     |     |      |     |     |     |     |     |     |     |     |     |
| Dimethylidooctadecylammonium bentonite.....            |     |     |     | 6   |     |      |     |     |     |     |     |     |     |     |     |
| Esteril GT.....                                        |     |     |     |     | 4   | 2.5  |     |     |     |     |     |     |     |     |     |
| Ratio of triazine compound to secondary thickener..... | 8:1 | 4:1 | 4:1 | 5:1 | 8:1 | 20:1 | 2:1 | 1:1 | 2:1 | 6:1 | 7:1 | 3:1 | 5:1 | 8:1 | 9:1 |

While our invention has been described with reference to various specific examples and embodiments, it will be understood that the invention is not limited to such examples and embodiments and may be variously practiced within the scope of the claims hereinafter made.

We claim:

1. A lubricating composition comprising a dispersion in a lubricating oil of a sufficient amount to thicken the lubricating oil to a grease consistency of a mixture of a 1,3,5-triazine compound melting above about 205° C. having the following formula:



wherein R and R<sub>1</sub> are selected from the group consisting of hydrogen, alkyl, aryl, alkaryl, aralkyl, cyanoalkyl, pyridyl, amino, hydroxy and mercapto radicals and wherein the alkyl radical contains from 1 to 4 carbon atoms, the alkyl portion of the alkaryl and aralkyl radicals contains from 1 to 2 carbon atoms and the alkyl portion of the cyanoalkyl radical contains from 1 to 8 carbon atoms, R and R<sub>1</sub> being unlike radicals when selected from the group consisting of amino, hydroxy and mercapto radicals and an organophilic siliceous oil thickening agent, the weight ratio of the 1,3,5-triazine compound to the organophilic siliceous material in said mixture being about 1:1 to about 20:1.

2. The lubricating composition of claim 1 wherein the combined 1,3,5-triazine compound and organophilic siliceous material comprises about 10 to 60 percent by weight of the total composition.

3. The lubricating composition of claim 1 wherein the lubricating oil is a polyorgano siloxane.

4. The lubricating composition of claim 1 wherein the organophilic siliceous oil thickening agent is a bentonite-organic base compound.

5. The lubricating composition of claim 1 wherein the organophilic siliceous oil thickening agent is an organophilic esteril comprising a supercolloidal substrate coated with —OR' groups, the substrate having a surface of silica and having a specific surface area of from 1 to 900 square meters per gram, the coating of —OR' groups being chemically bound to said silica and R' being a hydrocarbon radical of from 2 to 18 carbon atoms, wherein the carbon attached to oxygen is also attached to hydrogen.

6. A lubricating composition comprising a dispersion in a liquid polyorgano siloxane of a sufficient amount to thicken the polyorgano siloxane to a grease consistency of a mixture of a 1,3,5-triazine compound melting above about 205° C. having the following formula:



wherein R and R<sub>1</sub> are selected from the group consisting of hydrogen, alkyl, aryl, alkaryl, aralkyl, cyanoalkyl, pyridyl, amino, hydroxy and mercapto radicals and wherein the alkyl radical contains from 1 to 4 carbon atoms, the alkyl portion of the alkaryl and aralkyl radicals contains from 1 to 2 carbon atoms and the alkyl portion of the cyanoalkyl radical contains from 1 to 8 carbon atoms, R and R<sub>1</sub> being unlike radicals when selected from the group consisting of amino, hydroxy and mercapto radicals and an organophilic bentonite-organic base compound, the weight ratio of 1,3,5-triazine compound to the organophilic bentonite-organic base compound in said mixture being about 1:1 to about 20:1.

7. A lubricating composition comprising a dispersion in a lubricating oil of a sufficient amount to thicken the lubricating oil to a grease consistency of a mixture of a guanamine derivative melting above about 205° C. having the following formula:



wherein R<sub>1</sub> is selected from the group consisting of hydrogen, alkyl, aryl, alkaryl, aralkyl, cyanoalkyl, pyridyl, hydroxy and mercapto radicals and wherein the alkyl radical contains from 1 to 4 carbon atoms, the alkyl portion of the alkaryl and aralkyl radicals contains from 1 to 2 carbon atoms and the alkyl portion of the cyanoalkyl radical contains from 1 to 8 carbon atoms and an organophilic bentonite-organic base compound, the weight ratio of the guanamine derivative to the organophilic bentonite-organic base compound in said mixture being about 1:1 to about 20:1.

8. The lubricating composition of claim 7 wherein the guanamine derivative is benzoguanamine and the ben-

11

tonite-organic base compound is dimethyldicetylammmonium bentonite.

9. A lubricating composition comprising a dispersion in a liquid polyorgano siloxane of a sufficient amount to thicken the polyorgano siloxane to a grease consistency of a mixture of benzoguanamine and dimethyldicetylammonium bentonite wherein the weight ratio of benzoguanamine to dimethyldicetylammonium bentonite is between about 1:1 and about 20:1.

10. A lubricating composition comprising a dispersion in a liquid polyorgano siloxane of a sufficient amount to thicken the polyorgano siloxane to a grease consistency of a mixture of ammelide and dimethyldicetylammonium bentonite wherein the weight ratio of ammelide to dimethyldicetylammonium bentonite is between about 1:1 and about 20:1.

11. A lubricating composition comprising a dispersion in a liquid polyorgano siloxane of a sufficient amount to thicken the polyorgano siloxane to a grease consistency of a mixture of ammeline and dimethyldicetylammonium bentonite wherein the weight ratio of ammeline to dimethyldicetylammonium bentonite is between about 1:1 and about 20:1.

12. A lubricating composition comprising a dispersion in a liquid polyorgano siloxane of a sufficient amount of thicken the polyorgano siloxane to a grease consistency of a mixture of 2,4-dihydroxy-6-pyridyl-1,3,5-triazine and dimethyldicetylammonium bentonite wherein the weight ratio of 2,4-dihydroxy-6-pyridyl-1,3,5-triazine to dimethyldicetylammonium bentonite is between about 1:1 and about 20:1.

13. A lubricating composition comprising a dispersion in a liquid polyorgano siloxane of a sufficient amount to thicken the polyorgano siloxane to a grease consistency of a mixture of 2,4-dimercapto-6-amino-1,3,5-triazine and dimethyldicetylammonium bentonite wherein the weight ratio of 2,4-dimercapto-6-amino-1,3,5-triazine to dimethyldicetylammonium bentonite is between about 1:1 and about 20:1.

14. A lubricating composition comprising a dispersion in a liquid polyorgano siloxane of a sufficient amount to thicken the polyorgano siloxane to a grease consistency

12

of a mixture of a 1,3,5-triazine compound melting above about 205° C. having the following formula:



10 wherein R and R<sub>1</sub> are selected from the group consisting of hydrogen, alkyl, aryl, alkaryl, aralkyl, cyanoalkyl, pyridyl, amino, hydroxy and mercapto radicals and wherein the alkyl radical contains from 1 to 4 carbon atoms, the alkyl portion of the alkaryl and aralkyl radicals contains from 1 to 2 carbon atoms and the alkyl portion of the cyanoalkyl radical contains from 1 to 8 carbon atoms, R and R<sub>1</sub> being unlike radicals when selected from the group consisting of amino, hydroxy and mercapto radicals and an organophilic estersil, the weight ratio of the 1,3,5-triazine compound to the organophilic estersil in said mixture being about 1:1 to about 20:1, said organophilic estersil comprising a supercolloidal substrate coated with —OR' groups, the substrate having a surface of silica and having a specific surface area of 25 to 900 square meters per gram, the coating of —OR' groups being chemically bound to said silica and R' being a hydrocarbon radical of from 3 to 6 carbon atoms, wherein the carbon atom attached to oxygen is also attached to hydrogen.

30 15. The lubricating composition of claim 14 wherein the 1,3,5-triazine compound is benzoguanamine and the organophilic ester'sil is an amorphous silica coated with about 340 butoxy groups per 100 square millimicrons of surface.

**References Cited in the file of this patent**

UNITED STATES PATENTS

|           |               |               |
|-----------|---------------|---------------|
| 2,714,057 | Chenicek      | July 26, 1955 |
| 2,820,763 | Hughes et al. | Jan. 21, 1958 |
| 2,859,234 | Clem          | Nov. 4, 1958  |
| 2,879,229 | Stratton      | Mar. 24, 1959 |